

Aug. 22, 1939.

L. NAVIAS

2,170,692

ELECTRIC HEATER

Filed July 31, 1937

Fig. 1.



Fig. 2.



Fig. 3.



Inventor:  
Louis Navias,

by Harry E. Junkins  
His Attorney.

## UNITED STATES PATENT OFFICE

2,170,692

## ELECTRIC HEATER

Louis Navias, Schenectady, N. Y., assignor to  
General Electric Company, a corporation of  
New York

Application July 31, 1937, Serial No. 156,740

8 Claims. (Cl. 201—64)

This invention relates to electric heaters and, more particularly, to electric heaters of the sheathed type, the new feature being an improved insulating material.

5 This invention has particular application to electric heaters of the sheathed type such as described and claimed in the United States patent to C. C. Abbott, No. 1,367,341, dated February 1, 1921, and assigned to the same assignee as the 10 present invention. Briefly, this heater comprises a resistance element enclosed in a metallic sheath, and embedded in and supported in spaced relation to the sheath, by a dense, compact mass of heat-refractory, heat-conducting, electrically insulating material. It is to be understood, however, that this invention is not limited to the specific heater disclosed in this patent, but has more 15 general application.

The heat-refractory insulating material that 20 has found wide application in sheathed heating units is magnesium oxide, usually in finely-divided form. Heating units provided with this material for the most part have been quite satisfactory. However, for various reasons, important 25 among which is the change in the composition of the magnesia which results, for example, from absorption of moisture and gases, for instance carbon dioxide, the electrical resistance of the heater does not remain constant but decreases in 30 use. This reduces the life of the heater and, of course, is not so satisfactory as would be the case if the electrical resistance remained constant, or substantially so. To obviate this difficulty it has heretofore been proposed to use beryllium oxide 35 in lieu of magnesium oxide as the insulating medium in sheathed heating units. Beryllium oxide is comparatively expensive, costing at present at least about ten times as much as magnesium oxide and, in addition, certain disadvantages are 40 encountered in its use not heretofore known or appreciated.

It is an object of the present invention to provide an electric heater which has a more constant electric resistance during the life of the heater 45 than heretofore has been possible by the use of conventional insulating mediums.

Another object of the invention is to provide an electric heater containing heat-refractory, heat-conducting insulating material of improved electrical resistance.

Another object of the invention is to provide a method for improving the electrical resistance of fused magnesia. The scope of the invention also includes the product of such method.

55 Other and further objects of the invention will

be apparent to those skilled in the art as a reading of this specification proceeds.

In accordance with this invention, the resistance conductor of the heater is embedded in, and supported in spaced relation with the walls of 5 its sheath by a layer of insulating material comprising a fusion product of magnesium oxide and beryllium oxide, advantageously with the latter present in the initial mixture in an amount not substantially exceeding 10 per cent by weight 10 thereof.

For a more complete understanding of the invention attention is directed to the following description and the accompanying drawing in which Fig. 1 is a fragmentary view in elevation of an 15 electric heater embodying this invention, portions of the heater being shown in section so as to illustrate certain structural details; and Figs. 2 and 3 are graphs illustrating the results of electrical tests on insulating compositions of this invention.

Referring to Fig. 1 of the drawing, this invention is there shown in one form as applied to an electric heater of the type described and claimed in the above-mentioned Abbott Patent 20 No. 1,367,341.

As shown, the heater comprises a helical resistance conductor mounted within, and substantially centrally of a tubular metallic sheath 11. The resistance conductor preferably is formed 30 of a nickel-chromium alloy. The sheath also preferably is formed of an alloy consisting chiefly of nickel and chromium.

The resistance conductor 10 is surrounded by, and supported in spaced relation with the sheath 35 by a layer 12 of heat-refractory, heat-conducting, electrically insulating material comprising a product made by fusing together magnesium oxide and beryllium oxide in a manner such as more fully described hereinafter. This insulating material may be compacted in the sheath by any suitable means, for example, by reducing the diameter of the sheath after the resistance conductor and insulating medium have been assembled with the sheath. The reducing operation may be 40 accomplished by swaging or rolling.

The resistance conductor 10 has its ends secured to terminals 13 which, as shown, have their inner ends embedded in the insulating material 12 so as to be supported in spaced relation with 50 the sheath.

In preparing the insulating composition of this invention magnesia prepared from metallic magnesium or from certain grades of magnesite of a high degree of purity may be employed. The 55

magnesia component may be obtained, for example, by the hydration of pure magnesium metal in an autoclave. The hydroxide is converted into the oxide by heating in an electric muffle or other suitable furnace to a temperature of, for instance, about 650° to 850° C. Beryllium oxide which initially has been fired to a temperature of about 1450° to 1550° C. advantageously may be employed.

The dry magnesium and beryllium oxides in predetermined proportions are thoroughly mixed, the relative proportions thereof being dependent, for example, upon their purity and the particular characteristics desired in the end-product. For example, the proportions may vary from about 0.50 to 10 parts by weight of beryllium oxide to about 99.50 to 90 parts by weight of magnesium oxide. The use of a higher or lower ratio of beryllia to magnesia is not precluded. The essential point is to use such ratio of beryllia to magnesia as will impart optimum electrically insulating properties to the end-product. The mixed oxides then are heated to a temperature sufficient to convert the mixture to liquid state, for example to a temperature of about 3000° to 3500° C., resulting in a completely liquefied product or what also may be described as a product of complete liquefaction of the magnesia-beryllia mixture, as distinguished from a sintered product. Any other suitable means of bringing about an intimate association of beryllium and magnesium oxides in molten state may be employed.

The fusion (liquefaction) product is cooled. When cold (solidified) it is crushed and screened to a suitable particle size, for example, to a size such that substantially all of it passes through a U. S. Sieve Series No. 40 sieve. The comminuted material is treated to remove iron, for example by magnetic separation, after which it is fired out of contact with metal surfaces to a temperature of, for example, about 1100° C. to 1400° C. The fired product advantageously is sifted through a screen of suitable size, for example a 40-mesh screen, and then stored in containers until put into use.

An examination under a petrographic microscope of compositions prepared as hereinbefore described reveals that they comprise substantially pure isotropic periclase crystals, or fragments thereof; periclase crystals or fragments having anisotropic beryllia-magnesia eutectic attached to a surface thereof; periclase crystals or fragments having facing surfaces coated with, and connected by anisotropic beryllia-magnesia eutectic; and, sometimes, small particles of anisotropic beryllia-magnesia eutectic itself.

Fig. 2 shows graphically the results of tests of the average resistance, plotted against the logarithm of time, of units containing insulating compositions of the present invention in comparison with fused magnesia and beryllia alone as insulating media. In this figure graphs A and B represent the results of testing units containing beryllium oxide and fused magnesium oxide, respectively; and graphs C, D and E represent the results of testing units containing compositions prepared as herein described from mixtures of 2 per cent, 5 per cent and 10 per cent, respectively, of beryllium oxide and the remainder magnesium oxide prepared from metallic magnesia.

In making the test, which is in effect a life test with pure metal electrodes under isothermal conditions, a series of ten units, two for each sample, was prepared with hydrogen-annealed nickel 75 parts. All of the units were arranged in a bundle

having a thermocouple assembly at its center, and were heated uniformly throughout their entire length and during the whole period of test (72 hours) at a temperature of 982° C. (1800° F.). Measurements of resistance, accurate within 0.1 per cent, were made at intervals of 1, 7, 24, 46 and 72 hours. Although the resistances determined at any one particular time are entirely relative, and cannot be used to predict the values obtainable at any other time, it is to be noted that the best maintenance of resistance is shown by the composition produced from a mixture of 5 per cent beryllium oxide and 95 per cent magnesium oxide. The poorest maintenance of resistance is shown by the fused beryllium oxide. All the compositions of this invention which were tested maintain their initial resistance better than fused magnesium oxide or fused beryllium oxide. This is important from the standpoint of design and service use of an electric heating unit.

It is also to be noted that although fused beryllia has a higher electrical resistance both initially and after 1 hour's heating at 982° C., thereafter its resistance decreases rapidly. The highest resistance to the passage of electric current at the end of 7, 24, 46 and 72 hours' heating was shown by the composition made from a mixture of 2 per cent beryllia and 98 per cent magnesia.

Fig. 3 shows the results of electrical resistance tests on units containing different magnesites ignited or calcined to oxidic state and compositions prepared from mixtures containing varying percentages of beryllia with said magnesites. In preparing the compositions the results of tests on which are designated as F, G and H, magnesites designated below for convenience as 1, 2 and 3, respectively, were used. These magnesites upon analysis of ignited samples were found to have the following chemical compositions:

|                                                                         | 1         | 2         | 3         |
|-------------------------------------------------------------------------|-----------|-----------|-----------|
| SiO <sub>2</sub> .....                                                  | 0.024     | 1.24      | 1.51      |
| CaO.....                                                                | 1.7       | 1.23      | 1.24      |
| Fe <sub>2</sub> O <sub>3</sub> and Al <sub>2</sub> O <sub>3</sub> ..... | 0.025     |           |           |
| Fe <sub>2</sub> O <sub>3</sub> .....                                    |           | 0.028     | 0.018     |
| Al <sub>2</sub> O <sub>3</sub> .....                                    |           | 0.023     | 0.018     |
| MgO.....                                                                | Remainder | Remainder | Remainder |

Varying percentages of beryllia were mixed with the individual calcined magnesites. The individual mixture then was fused and further processed essentially in the same manner as hereinbefore described with reference to compositions utilizing magnesia prepared from metallic magnesium.

Graphs F and G were plotted from electrical resistance values of calcined magnesites 1 and 2, respectively, and of compositions prepared by fusing 2, 3 and 5 per cent beryllia with each of said calcined magnesites. Graph H was plotted from the resistance values of calcined magnesite 3 and of compositions prepared by fusing 1, 2, 3, 5 and 10 per cent beryllia with said magnesite. As shown by these graphs, a composition made from a mixture of 2 per cent beryllia and 98 per cent magnesia (from magnesite) has a higher electrical resistance than compositions utilizing other percentage proportions. Such a composition represents a preferred embodiment of this invention. All compositions of the present invention have practical usefulness as electrically insulating materials.

What I claim as new and desire to secure by Letters Patent of the United States is:

1. An electric heater comprising a metallic

- sheath, a resistance element encased by said sheath and between said resistance conductor and said sheath a layer of an insulating composition consisting of the comminuted solidified product of liquefaction of a mixture of magnesium oxide and beryllium oxide, the latter not exceeding substantially 10 per cent by weight of the whole. 5
2. An electric heater comprising a tubular metallic sheath, a resistance conductor within 10 said sheath and insulating material consisting of the comminuted solidified product of liquefaction of a mixture of about 0.5 per cent to 10 per cent by weight beryllium oxide and the remainder magnesium oxide, said insulating material being compacted within said sheath about said resistance conductor and supporting the latter in spaced relation with said sheath. 15
3. An electric heater comprising a tubular metallic sheath, a resistance conductor within 20 said sheath arranged centrally thereof and powdered, densely compacted insulating material consisting of the powdered solidified product of liquefaction of a mixture of about 0.5 per cent to 5 per cent by weight beryllium oxide and the 25 remainder magnesium oxide, said insulating material surrounding said resistance conductor and supporting the latter in spaced relation with said sheath. 30
4. An electric heater comprising a metallic sheath, a resistance conductor within said sheath and insulating material consisting of the comminuted solidified product of liquefaction of a mixture of approximately 98 parts by weight of magnesium oxide and approximately 2 parts by
- weight of beryllium oxide, said insulating material being compacted within said sheath about said resistance conductor and supporting the latter in spaced relation with said sheath. 5
5. An electrically insulating composition consisting of the comminuted solidified product of liquefaction of a mixture of magnesium oxide and beryllium oxide, the latter not exceeding substantially 10 per cent by weight of the whole. 10
6. The method of preparing a material especially adapted for use as insulation in electric heaters of the sheathed type which comprises forming a liquid mixture of magnesium oxide and not exceeding substantially 10 per cent by weight of the whole or beryllium oxide, cooling 15 the resultant mass, and comminuting the cooled mass. 15
7. The method which comprises forming a liquid mixture of magnesium oxide and from 0.5 to 10 per cent by weight of the whole of beryllium 20 oxide, cooling the resulting mass, comminuting the cooled mass, and heating the comminuted mass to a temperature of about 1100° to 1400° C. 20
8. The method which consists in thoroughly mixing, by weight, approximately 2 per cent 25 beryllium oxide with approximately 98 per cent magnesium oxide, heating the mixture to about 3000° to 3500° C. completely to liquefy it, cooling the liquefied product, comminuting the cooled product, treating the comminuted product to remove iron, and heating the thus treated product out of contact with metal surfaces to a temperature of about 1100° to 1400° C. 30

LOUIS NAVIAS.